# EUROPEAN PATENT SPECIFICATION

(11) **EP 1 564 019 B1**
(45) Date of publication and mention of the grant of the patent: **15.08.2007**
(21) Application number: 04405087.0
(22) Date of filing: 17.02.2004
(51) Int. Cl.: B41M 5/124, B41M 5/165

(54) **Copying sheet and method for creating or enhancing copying quality of a copying sheet**
Kopierblatt und Methode für das Verursachen oder das Erhöhen von Kopiequalität eines Kopierblattes
Feuille à copier et méthode pour créer ou augmenter la qualité de copie d'une feuille à copier

(43) Date of publication of application: 17.08.2005
(73) Proprietor: Sensient Imaging Technologies S.A., 1110 Morges (CH)
(72) Inventor: Boksanyi, Laszlo, 1025 St. Sulpice (CH); Mury, Pierre, 1008 Prilly (CH); Boissard, Christophe, 1870 Monthey (CH)
(74) Representative: Hepp, Dieter

(56) References cited:
- EP-A- 0 449 537
- EP-A- 0 629 511
- US-A- 3 682 682
- US-A- 4 761 397
- US-A- 4 783 438
- DATABASE WPI Section Ch, Week 200166 Derwent Publications Ltd., London, GB; Class G05, AN 2001-585007 XP002287831 & JP 2001 063260 A (TOPPAN MOORE KK) 13 March 2001 (2001-03-13)

## Description

The present invention is related to the field of especially pressure-sensitive copying sheets, and to coatings useful for the manufacture of such copying sheets.

Traditionally, pressure-sensitive copying sheets were based on a carbon wax coating, that was applied to the back of the sheet. A major drawback of such sheets was, that the carbon wax is sensitive to unwanted rubbing-off, resulting in a relatively dirty using characteristic. Moreover, the transferred carbon is delible and can be erased with relative ease and/or bleaches out.

Moreover, pressure- and/or heat-sensitive carbonless copying sheets are currently known in the art. These systems comprise a copying sheet (often referred to as CB) and a receiving sheet (often referred to as CF), which is separate from but may be connected to the copying sheet. The copying sheet is coated with a color agent on its back, e.g. a leuco dye. The receiving sheet is coated with a developer on its side directed to the coated side of the copying sheet. Color agent and/or developer may be provided in micro-encapsulated form, whereby the micro-capsules rupture under pressure such as applied by a typewriter head or a pencil. Both the color agent and developer are mostly transparent as long as separated from each other. However, upon contact of color agent and developer, an image is produced on the receiving sheet in correspondence to where pressure has been applied. Although such systems are frequently used, a major drawback is that the intensity and/or durability of the image on the receiving paper is not sufficient for some purposes.

In order to improve the copying-intensity of such a CB sheet, an additional layer of a dry carbon printing medium (i.e. an additional carbon wax coating as mentioned above) has been proposed by GB-A-2 197 668. When a suchlike coated sheet is used with a CF sheet the resulting copy is bolder than with a conventional CB sheet. However, the resulting transcription is prone to aging, i.e. the durability of the transcription on the CF sheet is not sufficient.

US 3,682,682 describes a pressure-sensitive copying material containing, on a paper sheet, a white pigment layer containing a finely divided solvent dye and, on the same or another sheet, microballoons containing a solvent for the solvent dye.

JP 2001-063260 discloses an invisible information holding body. Invisible information is carried by a developer ink layer, provided onto a solvent containing microcapsule ink layer and a dye containing microcapsule ink layer underneath.

US 4,783,438 discloses a partially pressure-sensitive recording paper, using an ink that has been applied partially, the ink having been prepared by uniformly dispersing microcapsules having a solution of a colorless electron-donating dyestuff as the core material.

EP-A-0 449 537 describes another pressure-sensitive copying paper. A subcoat of plastic pigment particles and a binder is provided beneath the microcapsule coating of otherwise conventional pressure-sensitive copying paper.

US 4,761,397 discloses a microcapsule sheet for pressure-sensitive copying, with a base paper having thereon a layer comprising microcapsules and synthetic polymer latex as a binder.

It is thus an object of the present invention to overcome the drawbacks of the mentioned prior art, especially to provide a copying sheet with enhanced quality and durability of transcription, which is easily and clean to handle.

These objects are solved by a copying sheet, a method of creating or enhancing the copying quality of a copying sheet, a kit of parts for manufacture of a copying sheet, and a copying kit comprising at least one copying sheet according to the invention as specified by the independent claims.

A copying sheet according to the invention comprises a first layer with an incorporated, especially micro-encapsulated solvent at least one especially micro-encapsulated color agent which is soluble in the solvent of the first layer, and a second layer containing at least one color agent, wherein upon an outer influence or action, the solvent of said first layer may penetrate said second layer at the position where the outer influence or action is applied, whereby said at least one color agent of the second layer is at least partially releasable by said solvent. Preferably, said first layer is applied by means of a commonly known coating process, whereas said second layer is preferably applied in a printing process, preferably an offset printing process.

Upon release of the at least one color agent of the second layer by the solvent, the color agent of the second layer is transferred to a receiving sheet, thereby producing an image corresponding to the applied outer action.

As used herein, the outer action preferably is pressure, especially applied by a type-writer key or a pencil. However, the basic principle of the invention is adaptable to various other outer actions such as e.g. heat. As used herein, micro-encapsulation is achieved by means of e.g. anionic microcapsules, e.g. made from urea-formaldehyde resin and/or melamine-formaldehyde resin or gelatin; the process of micro-encapsulation is well known to those of ordinary skill in the art and is disclosed e.g. in US 4,001,140; US 4,100,103; US 4,552,811 (incorporated herewith by reference). It is, however, obvious to the person of routine skill in the art that the invention may be used on the basis of any conventional copying sheet based on preferably microencapsulated solvent(s), that are known in the art.

According to the present invention, the first layer of the copying sheet comprises at least one additional, especially micro-encapsulated color agent, which is at least partially soluble, most preferably completely soluble in the solvent of the first layer. This additional color agent of the first layer is preferably co-micro-encapsulated with the solvent. However, it is also possible to provide separate micro-capsules of solvent and color agent. The first layer of the copying sheet, especially according to this embodiment of the invention, may be the same as those known for conventional carbon-less copying sheets, e.g. comprising a leuco dye as described above. The solvent is provided in an amount sufficient to provide for transfer of both the color agents of the first layer and the second layer to a receiving sheet.

Preferred solvents and/or liquid core materials incorporated in the first layer are known by the person of ordinary skill in the art, especially chosen from the group consisting of ethyldiphenylmethane, benzylxylene, alkyl biphenyls, dialkyl phtalates, alkylated naphtalenes, partially hydrogenated terphenyls, high-boiling straight or branched chain hydrocarbons, high molecular weight esters, high molecular weight branched or linear alcohols and mixtures thereof.

According to the present invention, an improvement of the intensity and durability of transcription of conventional carbon-less copying sheets can be achieved: the color agent of the second layer is released by the solvent incorporated in the first layer, thus enhancing the resulting in-intensity of transcription achievable with conventional carbonless copying sheets, e.g. comprising a leuco dye.

In a further embodiment of the invention, the second layer of the copying sheet comprises a printed ink, e.g. a nucleophilic ink. The ink is configured suchlike to be absorbed into the paper, thus allowing clean handling of the copying sheet. Preferably, the ink does not dry significantly by evaporation of solvents or chemical crosslinking reactions or the like. The ink needs to be chemically compatible with the solvent incorporated in the first layer, i.e. no accidental color development especially of the additional color agent of the first layer should occur. Especially preferred is the use of a desensitizing ink such as those disclosed in US 5,035,743 (incorporated herewith by reference): the nucleophilicity of such an ink on the one hand prevents the color agent of the first layer, e.g. a leuco dye, from being accidentally developed; color development thus only occurs upon contact with an especially acidic developer provided by a receiving sheet. On the other hand, the ink is chosen suchlike to liberate an additional color agent out of the second layer for enhancing transcription upon the solvent of the first layer penetrating the second layer. Preferably, the color agent of the second layer is independent from an additional developer, thus providing a means for transcription even in the absence of a receiving sheet carrying a developer; thus, conventional paper may be used for generating a transcription only depending on the color agent of the second layer.

Preferably, the ink comprises carbon black and/or other pigments as the color agent(s), at least one binder and at least one solvent; adaptation of both binder and solvent are within the routine practice of the person skilled in the art. The at least one binder is preferably chosen from phenolic resins, maleic resins, rosin-modified resins, alkylated resins, rosin ester resins or the like, or mixtures thereof. The at least one solvent is preferably chosen from mineral oils, glycols, vegetable oils, alcohols or the like, or mixtures thereof.

Such carbon black (e.g. Regal 400R Carbon Black, Cabot; or the like) and other pigments (e.g. DPP Rubine TR, Ciba; Paliogen Blue L 6495F, BASF; Heliogen Green L 9361, BASF; Red HFG, Clariant; Blue R 54, Clariant; or the like) are commonly available in various colors and may be incorporated in the ink as finely dispersed particles. According to an especially preferred embodiment, the ink comprises carbon black. The pigments are embedded within the other ingredients of the ink. For special applications, a dye might be additionally included into the ink as well.

In an especially advantageous embodiment, the second layer of the copying sheet comprises different color agents in different parts of the copying sheet. Differently colored sections of a resulting transcription may thus be easily achieved, thereby facilitating e.g. specific accentuation especially on transcription forms. For example, the transcription of a price on an order form or delivery form or a bill may be provided in a striking color, e.g. in red. Further applications in this respect are apparent to the person of routine skill in the art.

It is especially preferred, that said at least one color agent of the first layer (e.g. a leuco dye) is chosen suchlike to develop a color upon contact with an especially acidic developer, which may be provided by a receiving sheet. Moreover, but not necessarily, the color agent of the second layer may also be chosen suchlike that it's coloration gets more intense upon contact with an especially acidic developer. Especially dyes are known to be prone to a change of color depending on the pH, thus a development or enhancement of a dye-mediated color can be achieved upon contact with an especially acidic developer.

Typical developers to be used are common knowledge of the person of routine skill in the art, and are preferably chosen from the group consisting of acidic clays, acidic resins (e.g. phenolic resins) or salicylate developers (e.g. zinc salicylate developers), derivatives and salts and mixtures thereof.

Moreover, the invention is also related to a method of creating or enhancing the copying quality of a copying sheet, comprising the steps of:
(a) Providing a backing material, which is at least partially supplied with a first layer with an incorporated, especially micro-encapsulated solvent, and
(b) At least partially applying a second layer onto said first layer, wherein the second layer comprises at least one color agent, which is at least partially releasable by said solvent of the first layer.

The first layer comprises at least one additional, preferably co-micro-encapsulated color agent, which is at least partly soluble in said solvent of the first layer.

The second layer is preferably applied in a printing process, especially an offset printing process. The offset printing process easily allows for high-quality prints in thin layer thickness, preferably of about 1 to 3 µm. Moreover, offset printing is preferred because it is the most widespread and the most economical one especially in business form printing. Additionally, typical solvents used in offset printing processes are oils, which are also good solvents for typical resins used for coating of the pigments and/or carbon black particles.

It is especially advantageous e.g. for forms or the like that the second layer is applied suchlike to comprise two or more different color agents, separated from each other. Application of different second layers beside each others can be easily achieved in commonly used printing processes such as offset printing.

Moreover, the invention provides a kit of parts for manufacture of a copying sheet, comprising
(a) components, either separate or pre-mixed, for applying a first layer onto a backing layer, comprising an incorporated, especially micro-encapsulated solvent and at least one preferably co-micro-encapsulated color agent which is soluble in said solvent;
(b) components, either separate or premixed, for applying a second layer onto said first layer, containing at least one color agent, which is at least partially releasable by the solvent incorporated in the first layer.

Another aspect of the present invention is a copying kit, comprising at least one copying sheet according to the invention as described above and at least one receiving sheet, wherein the receiving sheet comprises an especially acidic developer, which generates a color upon transfer of said at least one color agent of the first layer and/or said color agent of the second layer to the receiving sheet.

A preferred embodiment of the invention will now be described in more detail by means of figure:
Fig. 1: general working principle.

According to the present invention shown in Figure 1, the copying sheet CB comprises a backing material (e.g. paper), a first layer 1 with a preferably micro-encapsulated solvent S and a preferably co-micro-encapsulated color agent 4 soluble in said solvent S and a second layer 2 containing at least one color agent 3. The second layer 2 is at least partially applied onto the first layer 1.

According to the present embodiment, embodiment, compositions of the first layer and the second layer are as follows:

For the backing material including the first layer, a conventional carbonless copying sheet such as Idem (ArjoWiggins) may be used.

The second layer, preferably applied in an offset printing process, comprises by means of example:

| | |
|---|---|
| 20% by weight: | carbon black (or pigment) |
| | |
| 23% by weight: | *Bremapal 3000* |
| | (phenolic resin, binder; Robert Kraemer GmbH & Co) |
| | |
| 42% by weight: | *Amine Polymer 2420* |
| | (Sensient; nucleophilic compound according to examples 1 and 2 of US 5, 035, 743, incorporated herewith by reference) |
| 8% by weight: | Calcium carbonate |
| | (optional pigment) |
| | |
| 7% by weight: | Polypropylene glycol |
| | (solvent, viscosity controller; a suitable MW range is to be chosen depending on the other ingredients and the envisaged application) |

A corresponding receiving sheet CF comprises a backing material 6, e.g. paper, and a layer comprising an especially acidic developer 5.

In use, the copying sheet CB and the receiving sheet CF are arranged suchlike that both the backing materials 6 of copying sheet CB and receiving sheet CF are directed outwards. Upon an outer influence or action, preferably pressure applied by a typewriter head or a pencil, to the backing material 6 of the copying sheet CB, the micro-encapsulated solvent S of the first layer 1 gets partially released by rupture of the micro-capsules where the pressure is applied. The released solvent S locally penetrates into the second layer 2, thereby releasing a color agent 3 out of the second layer 2. The color agent 3 of the second layer 2 develops an image in correspondence to the applied pressure upon contact with the especially acidic developer 5 on the receiving sheet CF. If pressure is applied to a section B of the copying sheet, where a second layer 2 was added, an image is produced on the receiving sheet. In contrast, no image on the receiving sheet CF is produced in those sections A, where no second layer 2 is applied to the copying sheet CB.

In the present invention, the first layer additionally also comprises a color agent 4, e.g. a leuco dye.

Besides this additional color agent, the formulation of the first layer remains the same as outlined above. If pressure is now applied to a section A of the copying sheet, an image is only produced on the receiving sheet CB by means of the color agent 4 of the first layer 1 getting in contact with the developer 5. However, if pressure is applied to a section B of the copying sheet CB, where an additional second layer is applied to the copying sheet CB, a more intense image is produced on the receiving sheet: The solvent S incorporated in the first layer 1 releases the color agent 3 from the second layer, and both the color agents 3 and 4 of second and first layer, respectively, are forming the image upon contact with the developer. Therefore, the second layer acts as an image enhancing layer.

For special needs, e.g. highlighting etc., different second layers 2 may be applied to different sections of the copying sheet CB. Thuslike, special colorations of the image can be easily achieved by a variation of the color agent 3 of only the second layer 2.

## Claims

1. A copying sheet (CB), comprising
• a first layer (1) with an incorporated, especially micro-encapsulated solvent (S), and at least one especially micro-encapsulated color agent (4), which is soluble in the solvent (S) of the first layer (1);
• a second layer (2) containing at least one color agent (3),
configured suchlike that upon an outer influence or action, preferably pressure, the solvent (S) of said first layer (1) may penetrate said second layer (2) at the position where the outer influence or action is applied, and whereby said at least one color agent of the second layer (3) is at least partially releasable by said solvent (S).

2. Copying sheet (CB) according to claim 1, wherein said additional color agent (4) of the first layer (1) is co-micro-encapsulated with the solvent (S).

3. Copying sheet (CB) according to one of claims 1 to 2, wherein said copying sheet (CB) is pressure-sensitive.

4. Copying sheet (CB) according to one of claims 1 to 3, wherein said second layer (2) comprises a printed ink.

5. Copying sheet (CB) according to claim 4, wherein the ink is nucleophilic.

6. Copying sheet (CB) according to one of claims 4 or 5, wherein said printed ink comprises a carbon dye.

7. Copying sheet (CB) according to one of claims 1 to 6, wherein said at least one color agent (4) of the first layer (1) is a leuco dye.

8. Copying sheet (CB) according to one of claims 1 to 7, wherein said solvent (S) of the first layer (1) is chosen from the group consisting of ethyldiphenylmethane, benzylxylene, alkyl biphenyls, dialkyl phtalates, alkylated naphtalenes, partially hydrogenated terphenyls, high-boiling straight or branched chain hydrocarbons, high molecular weight esters, high molecular weight branched or linear alcohols and mixtures thereof.

9. Copying sheet (CB) according to one of claims 1 to 8, wherein the second layer (2) comprises different color agents (3) in different parts of the copying sheet (CB).

10. Copying sheet (CB) according to one of claims 1 to 9, wherein said at least one color agent (4) of the first layer (1) and/or said color agent (3) of the second layer (2) is chosen suchlike to develop a color upon contact with an especially acidic developer (5).

11. Copying sheet (CB) according to claim 10, wherein said developer (5) is chosen from the group consisting of acidic clay, acidic resins such as phenolic resins or salicylate developers such as zinc salicylate developers, derivatives and salts and mixtures thereof.

12. A method of creating or enhancing the copying quality of a copying sheet (CB) especially according to one of claims 1 to 12, comprising the steps of:
• Providing a backing material (6), which is at least partially supplied with a first layer (1) with an incorporated, especially micro-encapsulated solvent (S), and at least onepreferably co-micro-encapsulated color agent (4), which is at least partly soluble in said solvent (S) of the first layer (1);
• At least partially applying a second layer (2) onto said first layer (1), wherein the second layer (2) comprises at least one color agent (3), which is at least partially releasable by said solvent (S) of the first layer (1).

13. A method according to claim 12, wherein the second layer (2) is applied in a printing process, especially an offset printing process.

14. A method according to one of claims 12 to 13, wherein the second layer (2) is applied suchlike to comprise two or more different color agents (3), separated from each other.

15. A kit of parts for manufacture of a copying sheet (CB) especially according to one of claims 1 to 12, comprising
• components, either separate or pre-mixed, for applying a first layer (1) onto a backing layer (6), comprising an incorporated, especially micro-encapsulated solvent (S) and at least one, especially microencapsulated color agent (4), which is soluble in said solvent (S);
• components, either separate or premixed, for applying a second layer (2) onto said first layer (1), containing at least one color agent (3), which is at least partially releasable by the solvent (S) incorporated in the first layer (1).

16. A copying kit, comprising at least one copying sheet (CB) according to one of claims 1 to 12 and at least one receiving sheet (CF), wherein the receiving sheet comprises an especially acidic developer (5), which generates a color upon transfer of said at least one color agent (4) of the first layer (1) and/or said color agent (3) of the second layer (2) to the receiving sheet (CF).

## Patentansprüche

1. Kopierblatt (CB), umfassend
• eine erste Schicht (1) mit einem eingelagerten, insbesondere mikroverkapselten Lösungsmittel (S) und mindestens einem im Lösungsmittel (S) der ersten Schicht (1) löslichen, insbesondere mikroverkapselten Farbmittel (4),
• eine zweite Schicht (2), enthaltend mindestens ein Farbmittel (3),
ausgebildet derart, daß das Lösungsmittel (S) der ersten Schicht (1) bei äußerer Einwirkung, vorzugsweise Druckausübung, am Einwirkungsort in die zweite Schicht (2) eindringen kann, wodurch das mindestens eine Farbmittel der zweiten Schicht (3) durch das Lösungsmittel (S) zumindest partiell freisetzbar ist.

2. Kopierblatt (CB) nach Anspruch 1, bei dem das zusätzliche Farbmittel (4) der ersten Schicht (1) zusammen mit dem Lösungsmittel (S) comikroverkapselt ist.

3. Kopierblatt (CB) nach einem der Ansprüche 1 bis 2, bei dem es sich um ein druckempfindliches Kopierblatt (CB) handelt.

4. Kopierblatt (CB) nach einem der Ansprüche 1 bis 3, bei dem die zweite Schicht (2) eine aufgedruckte Tinte umfaßt.

5. Kopierblatt (CB) nach Anspruch 4, bei dem die Tinte nukleophil ist.

6. Kopierblatt (CB) nach einem der Ansprüche 4 oder 5, bei dem die aufgedruckte Tinte einen Farbruß umfaßt.

7. Kopierblatt (CB) nach einem der Ansprüche 1 bis 6, bei dem es sich bei dem mindestens einen Farbmittel (4) der ersten Schicht (1) um einen Leukofarbstoff handelt.

8. Kopierblatt (CB) nach einem der Ansprüche 1 bis 7, bei dem das Lösungsmittel (S) der ersten Schicht (1) ausgewählt ist aus der Gruppe, bestehend aus Ethyldiphenylmethan, Benzylxylol, Alkylbiphenylen, Dialkylphthalaten, alkylierten Naphthalinen, teilhydrierten Terphenylen, schwersiedenden gerad-oder verzweigtkettigen Kohlenwasserstoffen, hochmolekularen Estern, hochmolekularen verzweigten oder linearen Alkoholen und deren Mischungen.

9. Kopierblatt (CB) nach einem der Ansprüche 1 bis 8, bei dem die zweite Schicht (2) unterschiedliche Farbmittel (3) in unterschiedlichen Bereichen des Kopierblatts (CB) umfaßt.

10. Kopierblatt (CB) nach einem der Ansprüche 1 bis 9, bei dem das mindestens eine Farbmittel (4) der ersten Schicht (1) und/oder das Farbmittel (3) der zweiten Schicht (2) so ausgewählt sind bzw. ist, daß sich bei Kontakt mit einem insbesondere sauren Entwickler (5) eine Farbe entwickelt.

11. Kopierblatt (CB) nach Anspruch 10, bei dem der Entwickler (5) ausgewählt ist aus der Gruppe, bestehend aus saurem Ton, sauren Harzen wie Phenolharzen oder Salicylat-Entwicklern wie Zinksalicylat-Entwicklern, Derivaten und Salze und Mischungen davon.

12. Verfahren zur Einstellung oder Verbesserung der Kopierqualität eines Kopierblatts (CB) insbesondere gemäß einem der Ansprüche 1 bis 11, bei dem man
• ein zumindest teilweise mit einer ersten Schicht (1) mit einem eingelagerten, insbesondere mikroverkapselten Lösungsmittel (S) und mindestens einem im Lösungsmittel (S) der ersten Schicht (1) zumindest teillöslichen, insbesondere co-mikroverkapselten Farbmittel (4) versehenes Trägermaterial (6) bereitstellt und
• die erste Schicht (1) zumindest teilweise mit einer zweiten Schicht (2) beaufschlagt, wobei die zweite Schicht (2) mindestens ein Farbmittel (3) umfaßt, welches durch das Lösungsmittel (S) der ersten Schicht (1) zumindest partiell freisetzbar ist.

13. Verfahren nach Anspruch 12, bei dem man die zweite Schicht (2) aufdruckt, insbesondere nach einem Offsetdruckverfahren.

14. Verfahren nach einem der Ansprüche 12 bis 13, bei dem man die zweite Schicht (2) so aufträgt, daß sie zwei oder mehr unterschiedliche Farbmittel (3) voneinander getrennt umfaßt.

15. Anordnung zur Herstellung eines Kopierblatts (CB) insbesondere gemäß einem der Ansprüche 1 bis 11, umfassend
• Komponenten, entweder getrennt oder vorgemischt, zur Applizierung einer ersten Schicht (1) auf einer Trägerschicht (6), umfassend ein eingelagertes, insbesondere mikroverkapseltes Lösungsmittel (S) und mindestens ein im Lösungsmittel (S) lösliches, insbesondere mikroverkapseltes Farbmittel (4);
• Komponenten, entweder getrennt oder vorgemischt, zur Applizierung einer zweiten Schicht (2) auf der ersten Schicht (1), enthaltend mindestens ein Farbmittel (3), welches durch das in der ersten Schicht (1) eingelagerte Lösungsmittel (S) zumindest partiell freisetzbar ist.

16. Kopieranordnung, umfassend mindestens ein Kopierblatt (CB) gemäß einem der Ansprüche 1 bis 11 und mindestens ein Empfangsblatt (CF), wobei das Empfangsblatt einen insbesondere sauren Entwickler (5) umfaßt, der bei Transfer des mindestens einen Farbmittels (4) der ersten Schicht (1) und/oder des Farbmittels (3) der zweiten Schicht (2) auf das Empfangsblatt (CF) eine Farbe erzeugt.

## Revendications

1. Feuille pour copie (CB), comprenant
• une première couche (1) comportant un solvant incorporé, tout spécialement microencapsulé (S), et au moins un agent coloré, en particulier microencapsulé, (4), qui est soluble dans le solvant (S) de la première couche (1);
• une deuxième couche (2) contenant au moins un agent coloré (3),
configurée de telle manière que, sous une influence ou une action extérieure, de préférence une pression, le solvant (S) de ladite première couche (1) puisse pénétrer ladite deuxième couche (2) à l'endroit où l'influence ou l'action extérieure est appliquée, et moyennant quoi ledit au moins un agent coloré de la deuxième couche (3) peut être au moins partiellement libéré par ledit solvant (S).

2. Feuille pour copie (CB) selon la revendication 1, dans laquelle ledit agent coloré supplémentaire (4) de la première couche (1) est co-microencapsulé avec le solvant (S).

3. Feuille pour copie (CB) selon l'une quelconque des revendications 1 et 2, dans laquelle ladite feuille pour copie (CB) est sensible à la pression.

4. Feuille pour copie (CB) selon l'une quelconque des revendications 1 à 3, dans laquelle ladite deuxième couche (2) comprend une encre imprimée.

5. Feuille pour copie (CB) selon la revendication 4, dans laquelle l'encre est nucléophile.

6. Feuille pour copie (CB) selon l'une quelconque des revendications 4 et 5, dans laquelle ladite encre imprimée comprend un colorant carboné.

7. Feuille pour copie (CB) selon l'une quelconque des revendications 1 à 6, dans laquelle ledit au moins un agent coloré (4) de la première couche (1) est un colorant leucodérivé.

8. Feuille pour copie (CB) selon l'une quelconque des revendications 1 à 7, dans laquelle ledit solvant (S) de la première couche (1) est choisi dans le groupe constitué par l'éthyldiphénylméthane, le benzylxylène, les alkylbiphényles, les phtalates de dialkyle, les naphtalènes alkylés, les terphényles partiellement hydrogénés, les hydrocarbures à chaîne droite ou ramifiée de point d'ébullition élevé, les esters de masse moléculaire élevée, les alcools ramifiés ou linéaires de masse moléculaire élevée et des mélanges de ceux-ci.

9. Feuille pour copie (CB) selon l'une quelconque des revendications 1 à 8, dans laquelle la deuxième couche (2) comprend des agents colorés (3) différents dans différentes parties de la feuille pour copie (CB).

10. Feuille pour copie (CB) selon l'une quelconque des revendications 1 à 9, dans laquelle ledit au moins un agent coloré (4) de la première couche (1) et/ou ledit agent coloré (3) de la deuxième couche (2) est choisi de manière à développer une couleur par contact avec un révélateur tout spécialement acide (5).

11. Feuille pour copie (CB) selon la revendication 10, dans laquelle ledit révélateur (5) est choisi dans le groupe constitué par l'argile acide, les résines acides telles que les résines phénoliques ou les révélateurs de type salicylate tels que les révélateurs de type salicylate de zinc, les dérivés et les sels et des mélanges de ceux-ci.

12. Procédé pour créer ou renforcer la qualité de copie d'une feuille pour copie (CB), tout spécialement selon l'une quelconque des revendications 1 à 11, comprenant les étapes consistant à :
• se procurer matériau de support (6), qui est au moins partiellement doté d'une première couche (1) comportant un solvant incorporé, tout spécialement microencapsulé (S), et d'au moins un agent coloré (4) de préférence co-microencapsulé, qui est au moins partiellement soluble dans ledit solvant (S) de la première couche (1) ;
• appliquer au moins partiellement une deuxième couche (2) sur ladite première couche (1), la deuxième couche (2) comprenant au moins un agent coloré (3), qui peut être au moins partiellement libéré par ledit solvant (S) de la première couche (1).

13. Procédé selon la revendication 12, dans lequel la deuxième couche (2) est appliquée dans un procédé d'impression, en particulier un procédé d'impression offset.

14. Procédé selon l'une quelconque des revendications 12 et 13, dans lequel la deuxième couche (2) est appliquée de manière à comprendre deux ou plus de deux agents colorés (3) différents, séparés les uns des autres.

15. Ensemble de pièces pour fabriquer une feuille pour copie (CB) tout spécialement selon l'une quelconque des revendications 1 à 11, comprenant
• des composants, séparés ou prémélangés, pour appliquer une première couche (1) sur une couche de support (6), comprenant un solvant incorporé, tout spécialement microencapsulé (S), et au moins un agent coloré (4), tout spécialement microencapsulé, qui est soluble dans ledit solvant (S);
• des composants, séparés ou prémélangés, pour appliquer une deuxième couche (2) sur ladite première couche (1), contenant au moins un agent coloré (3), qui peut être au moins partiellement libéré par le solvant (S) incorporé dans la première couche (1).

16. Nécessaire pour copie, comprenant au moins une feuille pour copie (CB) selon l'une quelconque des revendications 1 à 11 et au moins une feuille réceptrice (CF), dans lequel la feuille réceptrice comprend un révélateur tout spécialement acide (5), qui génère une couleur par transfert sur la feuille réceptrice (CF) dudit au moins un agent coloré (4) de la première couche (1) et/ou dudit agent coloré (3) de la deuxième couche (2).
